

## UNITED STATES PATENT OFFICE

2,440,330

IMPROVING THE FASTNESS OF DYED  
ORGANIC DERIVATIVE OF CELLU-  
LOSE TEXTILES BY IMPREGNATION  
WITH CYANAMIDE

Henry Dreyfus, London, England; Claude Bonnard, administrator of said Henry Dreyfus, deceased, assignor to Celanese Corporation of America, a corporation of Delaware

No Drawing. Application August 15, 1944, Serial No. 549,625. In Great Britain August 26, 1943

5 Claims. (Cl. 8—61)

1

This invention relates to the incorporation of difficultly soluble nitrogenous compounds in textile materials for various purposes, for example, to improve fastness of dyes, to impart affinity for acid dyes, to modify lustre, or to fix dyes, pigments, sizes and the like upon the material.

It is very convenient to be able to effect application of such nitrogenous compounds, or components from which the compounds can be prepared on the material, by a simple padding or other mechanical impregnation operation using an appropriate aqueous solution. However, many nitrogenous compounds useful for these purposes, or components from which they can be produced, are of such low solubility in water that it is difficult to apply the requisite proportion of substance in this way. Thus in the case of melamine, a substance useful for improving the resistance of colourations on cellulose acetate materials to combustion products of coal gas, the solubility in water at ordinary temperature is less than 0.5% and at 50° C. is only about 1%. Again, the solubility of di-cyandiamide in water at ordinary temperature is only of the order of 2%. In padding a textile material with a liquid it is not practicable to arrange to leave in the material much more than about its own weight of liquid. In the case of melamine, therefore, it is only practicable to incorporate in this way about 0.5% on the weight of the material by padding at ordinary temperatures.

It has been found that cyanamide can usefully be employed for preparing textile materials carrying such nitrogenous compounds difficultly soluble in water. Cyanamide is very soluble in water, even at ordinary temperatures, and by heat treatment, even at temperatures below 100° C., or reaction with an aldehyde, or both, can be converted into difficultly soluble nitrogenous compounds (including water-insoluble products).

Conveniently the cyanamide is applied to the textile material in the form of an aqueous solution, which may contain an acid, and the material then dried and heated to a temperature which will convert the cyanamide into a nitrogenous compound of but little solubility in water. For example the material may be heated at 90° to 150° C. As the cyanamide is very soluble in water it is easy to apply a substantial proportion, e. g. 5% or more, by a single impregnation with an aqueous solution and so to incorporate in the material a proportionately large amount of the soluble nitrogenous compound. The acid can be acetic or other organic acid.

An aqueous solution of cyanamide is conven-

2

iently prepared by extracting commercial calcium cyanamide with water at a fairly low temperature, say 40° C. or lower, filtering, passing carbon dioxide through the filtrate until the calcium is substantially precipitated as carbonate, again filtering, and then concentrating the filtrate at a low temperature, conveniently under reduced pressure. The concentration can be effected for instance at 40° C. under reduced pressure. Aqueous solutions of cyanamide of up to 40% strength can be obtained in this way.

The new process can be used for incorporating nitrogenous compounds in textile material for various purposes, for example any of those referred to above. The textile may be of natural or regenerated cellulose or of a cellulose ester or ether and in fabric, yarn, loose staple fibre, or other form.

The treatment may be applied for example to a cellulose ester or ether textile which has been coloured with a dye, e. g. a violet or blue amino-anthraquinone dye, which is insufficiently resistant to the action of combustion products of coal gas, so as to improve its resistance to this agency. Examples of such dyes are 1:4-diamino-anthraquinone and its N-alkyl and N-aryl derivatives, e. g. 1:4-di(methylamino)-anthraquinone, 1-methylamino-4-(beta-hydroxy-ethylamino)-anthraquinone, 1-amino-4-methylamino-anthraquinone and 1-amino-4-phenylamino-anthraquinone.

The invention is illustrated by the following example:

*Example*

35 A cellulose acetate fabric, dyed to a medium blue shade with 1-methylamino-4-beta-hydroxyethylaminoanthraquinone, is padded with a 6% aqueous solution of cyanamide containing 50 cc. of glacial acetic acid per litre, the padding being conducted so that the fabric retains about its own weight of the solution. The fabric is then dried and baked for 20 minutes at 130° C. As compared with the untreated dyeing the treated dyeing possesses a considerably increased resistance to the combustion products of coal gas.

Having described my invention, what I desire to secure by Letters Patent is:

1. Process for improving the color fastness of dyed textile material which comprises impregnating a dyed textile material having a basis of an organic derivative of cellulose with an aqueous solution of cyanamide and then drying and heating the impregnated material until a difficultly soluble nitrogenous compound is formed.
- 55 2. Process for improving the color fastness of

dyed textile material which comprises impregnating a dyed textile material having a basis of an organic derivative of cellulose with an aqueous solution of cyanamide, drying the impregnated material and then heating at a temperature of 110-150° C., until a difficultly soluble nitrogenous compound is formed.

3. Process for improving the color fastness of dyed textile material which comprises impregnating a dyed textile material having a basis of cellulose acetate with an aqueous solution of cyanamide and then drying and heating the impregnated material until a difficultly soluble nitrogenous compound is formed.

4. Process for improving the color fastness of dyed textile material which comprises impregnating a dyed textile material having a basis of cellulose acetate with an aqueous solution of cyanamide, drying the impregnated material and then heating at a temperature of 110-150° C., until a difficultly soluble nitrogenous compound is formed.

5. Process for improving the color fastness of dyed textile material which comprises impregnating with an aqueous solution of cyanamide, a

cellulose acetate textile material colored with an amino-anthraquinone dyestuff, drying the material and heating it at a temperature of 110-150° C., until a difficultly soluble nitrogenous compound is formed.

HENRY DREYFUS.

REFERENCES CITED

The following references are of record in the 10 file of this patent:

UNITED STATES PATENTS

|    | Number    | Name    | Date          |
|----|-----------|---------|---------------|
| 15 | 1,985,248 | Ellis   | Dec. 25, 1934 |
|    | 2,123,152 | Rivat   | July 5, 1938  |
|    | 2,176,506 | McNally | Oct. 17, 1939 |
|    | 2,234,889 | Boulton | Mar. 11, 1941 |
|    | 2,234,905 | Tallis  | Mar. 11, 1941 |
|    | 2,247,353 | Auer    | July 1, 1941  |
| 20 | 2,318,464 | Cameron | May 4, 1943   |
|    | 2,331,670 | Ericks  | Oct. 12, 1943 |

FOREIGN PATENTS

|    | Number  | Country       | Date          |
|----|---------|---------------|---------------|
| 25 | 537,964 | Great Britain | July 15, 1941 |